

P. T. JACKSON, JR.  
REINFORCED PAPER STRIP FOR BOX CORNERS AND OTHER PURPOSES.  
APPLICATION FILED FEB. 2, 1918.

1,278,935.

Patented Sept. 17, 1918.



Fig. 1



Fig. 3

Fig. 2

3 Inventor:  
Patrick Tracy Jackson, Jr.  
by Robert Fairus.  
Attorney

# UNITED STATES PATENT OFFICE.

PATRICK TRACY JACKSON, JR., OF CAMBRIDGE, MASSACHUSETTS, ASSIGNOR TO PAPER PRODUCTS MACHINE COMPANY, OF BOSTON MASSACHUSETTS, A CORPORATION OF MASSACHUSETTS.

## REINFORCED PAPER STRIP FOR BOX-CORNERS AND OTHER PURPOSES.

1,278,935.

Specification of Letters Patent. Patented Sept. 17, 1918.

Application filed February 2, 1918. Serial No. 215,181.

*To all whom it may concern:*

Be it known that I, PATRICK TRACY JACKSON, Jr., a citizen of the United States, residing at Cambridge, county of Middlesex,

5 and State of Massachusetts, have invented an Improvement in Reinforced Paper Strips for Box-Corners and other Purposes, of which the following description, in connection with the accompanying drawings, is 10 a specification, like characters on the drawings representing like parts.

The invention to be hereinafter described relates to reinforced paper fabrics adapted for adhesive engagement with objects.

15 Among other uses the fabric serves effectively for uniting the sides of boxes, reinforcing the corners thereof, and for sealing boxes or the wrappers of boxes and other containers or articles.

20 Heretofore paper fabrics of this general class have been reinforced by spaced threads or strings which have been spun or twisted into a continuous filament, and such threads or strings have been applied either trans- 25 versely or longitudinally to the fabric to be reinforced; and the fabric has had a gum coating for securing the same to articles. There are, however, certain objections to these fabrics. The spun or twisted threads

30 or strings necessarily have considerable body or thickness which adds materially to the stiffness of the fabric, and prevents free flexibility of the fabric, prevents the fabric from conforming intimately with the con- 35 tour of the article to which it is applied, and consequently prevents adhesive engagement of the gummed face of the fabric with the article throughout the area of said gummed face. The body or thickness of the spun

40 or twisted threads produces alternating grooves and ridges on the surface of the fabric, which are liable to be scraped and worn in use and cause rupture of the paper at said ridges. Also the spun and twisted 45 threads have been spaced substantial distances apart, so that substantial areas of the paper are left without reinforcement.

The purpose of the present invention, therefore, is to provide a reinforced fabric 50 which will overcome the above and other objections to reinforced fabrics now in use.

The character of the invention will be best understood from the following description of one good form thereof shown in the accompanying drawing, wherein:

55

Figure 1 is a plan view of a strip of paper or fabric having a gummed external face and a series of unspun fibers adhesively secured to the opposite face of the paper or fabric;

60

Fig. 2 is a plan view of a reinforced fabric having an external gummed face and comprising two plies of paper having unspun fibers secured by an adhesive between them; and

65

Fig. 3 is a section taken on line 3—3 of Fig. 2.

Referring to the drawing, 1 (Fig. 1) represents a strip of paper or other fabric to be reinforced or strengthened and having an 70 external gum coating 3 on one face thereof, which may be a vegetable or animal gum normally dry, but rendered adhesive on moistening the same, so that the fabric may be readily secured to the article desired.

75

The paper or fabric is reinforced or strengthened by the application to the opposite face from the gum coating, of unspun fibers 5 which may be any well known fibers, either animal or vegetable, but preferably 80

the latter, such, for example, as flax, sisal, hemp, cotton, waste, jute, and the like. The fiber is first "prepared" in the usual manner according to the character of fiber employed, which has the effect of laying the fibers in a 85

general parallel relation, the word parallel being herein used in a general though not strict sense, but since the machines and processes for preparing fibers are well known to those skilled in the art, and the invention 90

does not relate thereto, detailed description of these machines and processes is unnecessary herein. The unspun fibers thus prepared, are then applied to the paper strip or fabric transversely thereto, that is, the 95

longitudinal or lengthwise dimension of the fibers extends generally cross-wise or transversely of the strip. A suitable adhesive is applied to the face of the strip, ordinarily previously to placing thereon the series of 100 unspun fibers. It is desirable in some cases that this adhesive shall render the strip

waterproof, and therefore, in the present instance, an adhesive coating 7 of black asphaltum or other suitable waterproof adhesive is applied to the paper, and the fibers 5 secured thereby to the paper. The unspun fibers may be applied to the strip as it is supplied from a paper making machine, or as the strip is supplied from a suitable roll.

The length of the individual fibers may be 10 less than the width of the fabric to be reinforced thereby. In such case, end portions such as indicated at 9 of transversely extending fibers overlap, the construction being such that overlapping ends of fibers in 15 different portions of the paper fabric are out of line with each other longitudinally of the fabric. As a consequence, no line of weakness is formed in the longitudinal direction of the fabric.

20. It may sometimes be desirable to protect the reinforcing fibers on account of their delicate nature. For this purpose a strip 11 of paper or fabric may be opposed to the strip 1 described, the construction being such 25 that the series of transversely extending fibers may be secured by the adhesive between two plies of fabric as represented in Figs. 2 and 3. The series of delicate fibers may be in such closely adjacent relation that they will 30 constitute a sheet which will reinforce the ply or plies of paper substantially throughout the area thereof without substantial zones or spaces of weakness between them, such as characterized the strip, referred to, 35 which is reinforced by spun or twisted threads or strings. The fabric reinforced by the unspun fibers does not produce on the surface of the fabric the unsightly, objectionable ridges and grooves which always 40 characterize a fabric reinforced by the spun and twisted threads or strings, but on the contrary, the fabric is smooth and homogeneous throughout. This smooth quality of the fabric enables the same to be readily 45 wound evenly and uniformly on rolls, thereby facilitating the marketing and use thereof.

As stated, the fabric reinforced as described, is adapted among other uses, for reinforcing box corners. In applying the reinforced strip thereto, a suitable length may be unwound from a roll and the gummed face of the strip may be moistened and adhesively secured to the box corner with the 50 unspun fibers extending transversely to the corner. Thus, the fibers are placed in tension across the corner and furnish the maximum reinforcement in the direction required. The fabric reinforced by the delicate unspun 55 fibers, furnishes an effective reinforcement or binder while retaining the desirable flexible quality of the fabric which enables the latter to conform intimately to the article to which it is applied, and thus the gummed face of the fabric may intimately, adhesively 60

engage the article throughout the area of said fabric and insure permanent reinforcement thereof.

It will be understood that the reinforced fabric described is not restricted to its use 70 for strengthening box corners, but that it may be applied to many other uses.

The invention is not limited to the specific embodiment shown, but various deviations may be made therefrom without departing 75 from the spirit and scope of the appended claims.

What is claimed is:—

1. As an article of manufacture, a reinforced or strengthened fabric for adhesive 80 engagement with objects, comprising a paper strip, an external gum coating on a face of said strip and normally dry, but rendered adhesive on moistening the same, and a series of closely adjacent reinforcing or 85 strengthening unspun fibers with their longitudinal dimension extending transversely of the fabric in general parallel relation.

2. As an article of manufacture, a reinforced or strengthened fabric for adhesive 90 engagement with objects, comprising a paper strip, an external gum coating on a face of said strip and normally dry, but rendered adhesive on moistening the same, a waterproof adhesive on the opposite face of said 95 strip, and a series of closely adjacent strengthening unspun fibers secured by said waterproof adhesive to said strip with their longitudinal dimension extending transversely of the fabric. 100

3. As an article of manufacture, a reinforced or strengthened fabric for adhesive engagement with objects, comprising two plies of paper, an external gum coating on a face of one of said plies of paper and normally dry, but rendered adhesive on moistening the same, an adhesive layer between said plies of paper, and a series of closely adjacent strengthening unspun fibers between said plies of paper and secured thereto 105 by said adhesive, said fibers having their longitudinal dimensions extending transversely of the fabric. 110

4. As an article of manufacture, a reinforced or strengthened fabric for adhesive 115 engagement with objects, comprising two plies of paper, an external gum coating on a face of one of said plies of paper and normally dry, but rendered adhesive on moistening the same, a waterproof adhesive layer 120 between said plies of paper, and a sheet of closely adjacent strengthening unspun fibers between said plies of paper and secured thereto by said waterproof adhesive, said fibers having their longitudinal dimension 125 extending transversely of the fabric in general parallel relation.

5. As an article of manufacture, a reinforced or strengthened paper fabric for adhesive engagement with objects, comprising 130

a paper strip, an external gum coating on a face of said strip and normally dry, but rendered adhesive on moistening the same, and a series of unspun fibers with the longitudinal dimension thereof extending transversely of the paper strip, the ends of transversely extending fibers being disposed out of line longitudinally of the paper strip to avoid lines of weakness longitudinally of the strip, and an adhesive for securing said fibers to said strip.

In testimony whereof I have signed my name to this specification.

PATRICK TRACY JACKSON, Jr.